



US007384717B2

(12) **United States Patent**  
Dinh et al.

(10) **Patent No.:** US 7,384,717 B2  
(45) **Date of Patent:** Jun. 10, 2008

(54) **PHOTORECEPTOR WITH IMPROVED  
OVERCOAT LAYER**

(75) Inventors: **Kenny-Tuan T Dinh**, Webster, NY (US); **John F Yanus**, Webster, NY (US); **Kendra M Giza**, Webster, NY (US); **James R Backus**, Rochester, NY (US); **T Edwin Freeman**, Woodstock, GA (US); **Markus R Silvestri**, Fairport, NY (US); **Michael L Mehan**, Rochester, NY (US)

(73) Assignee: **Xerox Corporation**, Norwalk, CT (US)

(\*) Notice: Subject to any disclaimer, the term of this patent is extended or adjusted under 35 U.S.C. 154(b) by 361 days.

(21) Appl. No.: 11/234,275

(22) Filed: Sep. 26, 2005

(65) **Prior Publication Data**

US 2007/0072101 A1 Mar. 29, 2007

(51) **Int. Cl.**  
**G03G 5/147** (2006.01)

(52) **U.S. Cl.** 430/66; 430/132

(58) **Field of Classification Search** 430/66, 430/132

See application file for complete search history.

(56) **References Cited**

U.S. PATENT DOCUMENTS

3,121,006 A 2/1964 Middleton et al.

|                   |         |                          |
|-------------------|---------|--------------------------|
| 4,050,935 A       | 9/1977  | Limburg et al.           |
| 4,281,054 A       | 7/1981  | Horgan et al.            |
| 4,297,425 A       | 10/1981 | Pai et al.               |
| 4,298,697 A       | 11/1981 | Baczec et al.            |
| 4,338,390 A       | 7/1982  | Lu                       |
| 4,457,994 A       | 7/1984  | Pai et al.               |
| 4,560,635 A       | 12/1985 | Hoffend et al.           |
| 4,599,286 A       | 7/1986  | Limburg et al.           |
| 4,871,634 A       | 10/1989 | Limburg et al.           |
| 5,149,609 A *     | 9/1992  | Yu et al. .... 430/58.7  |
| 5,368,967 A       | 11/1994 | Schank et al.            |
| 5,418,107 A       | 5/1995  | Nealey et al.            |
| 5,681,679 A       | 10/1997 | Schank et al.            |
| 5,702,854 A       | 12/1997 | Schank et al.            |
| 5,709,974 A       | 1/1998  | Yuh et al.               |
| 5,976,744 A       | 11/1999 | Fuller et al.            |
| 6,004,709 A       | 12/1999 | Renfer et al.            |
| 2007/0134573 A1 * | 6/2007  | Yanus et al. .... 430/66 |

OTHER PUBLICATIONS

Technical Data Sheet for "SOVERMOL® 750," Cognis, May 23, 2005.

Technical Data Sheet for "DESMOPHEN® 800," Bayer, May 12, 2004.

\* cited by examiner

Primary Examiner—Hoa Van Le

(74) Attorney, Agent, or Firm—Oliff & Berridge, PLC

(57) **ABSTRACT**

An electrophotographic imaging member includes a substrate, a charge generating layer, a charge transport layer, and an overcoating layer, the overcoating layer including a cured polyester polyol or cured acrylated polyol film forming resin and a charge transport material.

**25 Claims, No Drawings**

## PHOTORECEPTOR WITH IMPROVED OVERCOAT LAYER

### BACKGROUND

This disclosure relates to electrophotographic imaging members and, more specifically, to layered photoreceptor structures with an improved overcoat layer. In particular, this disclosure relates to electrophotographic imaging members with an improved overcoat layer comprising, as a binder material, a polyester-polyol or polyether-ester polyol, and a hole transporting molecule. This disclosure also relates to processes for making and using the imaging members.

Electrophotographic imaging members, i.e. photoreceptors, typically include a photoconductive layer formed on an electrically conductive substrate. The photoconductive layer is an insulator in the dark so that electric charges are retained on its surface. Upon exposure to light, the charge is dissipated.

Many advanced imaging systems are based on the use of small diameter photoreceptor drums. The use of small diameter drums places a premium on photoreceptor life. A major factor limiting photoreceptor life in copiers and printers, is wear. The use of small diameter drum photoreceptors exacerbates the wear problem because, for example, 3 to 10 revolutions are required to image a single letter size page. Multiple revolutions of a small diameter drum photoreceptor to reproduce a single letter size page can require up to 1 million cycles from the photoreceptor drum to obtain 100,000 prints, a desirable goal for commercial systems.

For low volume copiers and printers, bias charging rolls (BCR) are desirable because little or no ozone is produced during image cycling. However, the micro corona generated by the BCR during charging, damages the photoreceptor, resulting in rapid wear of the imaging surface, e.g., the exposed surface of the charge transport layer. For example, wear rates can be as high as about 16 microns per 100,000 imaging cycles. Similar problems are encountered with bias transfer roll (BTR) systems. One approach to achieving longer photoreceptor drum life is to form a protective overcoat on the imaging surface, e.g. the charge transporting layer of a photoreceptor. This overcoat layer must satisfy many requirements, including transporting holes, resisting image deletion, resisting wear, avoidance of perturbation of underlying layers during coating.

Various overcoats employing alcohol soluble polyamides have been proposed in the prior art. One of the earliest ones is an overcoat comprising an alcohol soluble polyamide without any methyl methoxy groups (Elvamide) containing N,N'-diphenyl-N,N'-bis(3-hydroxyphenyl)-[1,1'-biphenyl]-4,4'-diamine. This overcoat is described in U.S. Pat. No. 5,368,967, the entire disclosure thereof being incorporated herein by reference. Although this overcoat had very low wear rates in machines employing corotrons for charging, the wear rates were higher in machines employing BCR. A cross linked polyamide overcoat overcame this shortcoming. This overcoat comprised a cross linked polyamide (e.g. Luckamide) containing N,N'-diphenyl-N,N'-bis(3-hydroxyphenyl)-[1,1'-biphenyl]-4,4'-diamine. In order to achieve cross linking of the polyamide polymer, Luckamide, having methyl methoxy groups was employed along with a catalyst such as oxalic acid. This tough overcoat is described in U.S. Pat. No. 5,702,854, the entire disclosure thereof being incorporated herein by reference. With this overcoat, very low wear rates were obtained in machines employing bias charging rolls (BCR) and Bias Transfer Rolls (BTR). Durable photoreceptor overcoatings containing cross linked

polyamide (e.g. Luckamide) containing N,N'-diphenyl-N, N'-bis(3-hydroxyphenyl)-[1,1'-biphenyl]-4,4'-diamine (DHTBD) (Luckamide-DHTBD) have been prepared using oxalic acid and trioxane to improve photoreceptor life by at least a factor of 3 to 4. Such improvement in the bias charging roll (BCR) wear resistance involved crosslinking of Luckamide under heat treatment, e.g. 110° C.-120° C. for 30 minutes. However, adhesion of this overcoat to certain photoreceptor charge transport layers, containing certain polycarbonates (e.g., Z-type 300) and charge transport materials (e.g., bis-N,N-(3,4-dimethylphenyl)-N-(4-biphenyl) amine and N,N'-diphenyl-N,N'-bis(3-methylphenyl)-[1,1'-biphenyl]-4,4'-diamine) is greatly reduced under such drying conditions. On the other hand, under drying conditions of below about 110° C., the overcoat adhesion to the charge transport layer was good, but the overcoat had a high rate of wear. Thus, there was an unacceptably small drying conditions window for the overcoat to achieve the targets of both adhesion and wear rate.

U.S. Pat. No. 5,702,854 describes an electrophotographic imaging member including a supporting substrate coated with at least a charge generating layer, a charge transport layer and an overcoating layer, said overcoating layer comprising a dihydroxy arylamine dissolved or molecularly dispersed in a crosslinked polyamide matrix. The overcoating layer is formed by crosslinking a crosslinkable coating composition including a polyamide containing methoxy methyl groups attached to amide nitrogen atoms, a crosslinking catalyst and a dihydroxy amine, and heating the coating to crosslink the polyamide. The electrophotographic imaging member may be imaged in a process involving uniformly charging the imaging member, exposing the imaging member with activating radiation in image configuration to form an electrostatic latent image, developing the latent image with toner particles to form a toner image, and transferring the toner image to a receiving member.

U.S. Pat. No. 5,681,679 discloses a flexible electrophotographic imaging member including a supporting substrate and a resilient combination of at least one photoconductive layer and an overcoating layer, the at least one photoconductive layer comprising a hole transporting arylamine siloxane polymer and the overcoating comprising a crosslinked polyamide doped with a dihydroxy amine. This imaging member may be utilized in an imaging process including forming an electrostatic latent image on the imaging member, depositing toner particles on the imaging member in conformance with the latent image to form a toner image, and transferring the toner image to a receiving member.

U.S. Pat. No. 6,004,709 discloses an allyloxy polyamide composition, the allyloxy polyamide being represented by a specific formula. The allyloxy polyamide may be synthesized by reacting an alcohol soluble polyamide with formaldehyde and an allyl alcohol. The allyloxy polyamide may be cross linked by a process selected from the group consisting of (a) heating an allyloxy polyamide in the presence of a free radical catalyst, and (b) hydrosilation of the double bond of the allyloxy group of the allyloxy polyamide with a silicon hydride reactant having at least 2 reactive sites. A preferred article comprises a substrate, at least one photoconductive layer, and an overcoat layer comprising a hole transporting hydroxy arylamine compound having at least two hydroxy functional groups, and a cross linked allyloxy polyamide film forming binder. A stabilizer may be added to the overcoat.

U.S. Pat. No. 5,976,744 discloses an electrophotographic imaging member is disclosed including a supporting sub-

strate coated with at least one photoconductive layer, and an overcoating layer, the overcoating layer including a hydroxy functionalized aromatic diamine and a hydroxy functionalized triarylamine dissolved or molecularly dispersed in a crosslinked acrylated polyamide matrix, the hydroxy functionalized triarylamine being a compound different from the polyhydroxy functionalized aromatic diamine. The overcoating layer is formed by coating. The electrophotographic imaging member may be imaged in a process.

U.S. Pat. No. 5,709,974 discloses an electrophotographic imaging member including a charge generating layer, a charge transport layer and an overcoating layer, the transport layer including a charge transporting aromatic diamine molecule in a polystyrene matrix and the overcoating layer including a hole transporting hydroxy arylamine compound having at least two hydroxy functional groups and a polyamide film forming binder capable of forming hydrogen bonds with the hydroxy functional groups of the hydroxy arylamine compound. This imaging member is utilized in an imaging process.

U.S. Pat. No. 5,368,967 discloses an electrophotographic imaging member comprising a substrate, a charge generating layer, a charge transport layer, and an overcoat layer comprising a small molecule hole transporting arylamine having at least two hydroxy functional groups, a hydroxy or multihydroxy triphenyl methane and a polyamide film forming binder capable of forming hydrogen bonds with the hydroxy functional groups the hydroxy arylamine and hydroxy or multihydroxy triphenyl methane. This overcoat layer may be fabricated using an alcohol solvent. This electrophotographic imaging member may be utilized in an electrophotographic imaging process. Specific materials including Elvamide polyamide and N,N'-diphenyl-N,N'-bis(3-hydroxyphenyl)-[1,1'-biphenyl]-4,4'-diamine and bis-[2-methyl-4-(N-2-hydroxyethyl-N-ethyl-aminophenyl)]-phenylmethane are disclosed in this patent.

U.S. Pat. No. 4,871,634 discloses an electrostaeographic imaging member which contains at least one electrophotocductive layer, the imaging member comprising a photo-generating material and a hydroxy arylamine compound represented by a certain formula. The hydroxy arylamine compound can be used in an overcoating with the hydroxy arylamine compound bonded to a resin capable of hydrogen bonding such as a polyamide possessing alcohol solubility.

U.S. Pat. No. 4,297,425 discloses a layered photosensitive member comprising a generator layer and a transport layer containing a combination of diamine and triphenyl methane molecules dispersed in a polymeric binder.

U.S. Pat. No. 4,050,935 discloses a layered photosensitive member comprising a generator layer of trigonal selenium and a transport layer of bis(4-diethylamino-2-methylphenyl) phenylmethane molecularly dispersed in a polymeric binder.

U.S. Pat. No. 4,457,994 discloses a layered photosensitive member is disclosed comprising a generator layer and a transport layer containing a diamine type molecule dispersed in a polymeric binder and an overcoat containing triphenyl methane molecules dispersed in a polymeric binder.

U.S. Pat. No. 4,281,054 discloses an imaging member comprising a substrate, an injecting contact, or hole injecting electrode overlying the substrate, a charge transport layer comprising an electrically inactive resin containing a dispersed electrically active material, a layer of charge generator material and a layer of insulating organic resin overlying the charge generating material. The charge transport layer can contain triphenylmethane.

U.S. Pat. No. 4,599,286 discloses an electrophotographic imaging member comprising a charge generation layer and

a charge transport layer, the transport layer comprising an aromatic amine charge transport molecule in a continuous polymeric binder phase and a chemical stabilizer selected from the group consisting of certain nitrone, isobenzofuran, hydroxyaromatic compounds and mixtures thereof. An electrophotographic imaging process using this member is also described.

U.S. Pat. No. 5,418,107 discloses a process for fabricating an electrophotographic imaging member including providing a substrate to be coated, forming a coating comprising photoconductive pigment particles having an average particle size of less than about 0.6 micrometer dispersed in a solution of a solvent comprising n-alkyl acetate having from 3 to 5 carbon atoms in the alkyl group and a film forming polymer consisting essentially of a film forming polymer having a polyvinyl butyral content between about 50 and about 75 mol percent, a polyvinyl alcohol, content between about 12 and about 50 mol percent, and a polyvinyl acetate content is between about 0 to 15 mol percent, the photoconductive pigment particles including a mixture of at least two different phthalocyanine pigment particles free of vanadyl phthalocyanine pigment particles, drying the coating to remove substantially all of the alkyl acetate solvent to form a dried charge generation layer comprising between about 50 percent and about 90 percent by weight of the pigment particles based on the total weight of the dried charge generation layer, and forming a charge transport layer.

Despite these various approaches, there remains a need for improved overcoat layer design, to provide increased wear resistance and resistance to moisture, such as humidity, and the like. A need also exists for improved overcoat layer design, to provide hard yet flexible layers that are more resistant to cracking. For example, the art has previously provided a range of hard overcoating layer materials. However, such overcoat layers are typically prone to cracking, especially during use, as well as humidity. Both effects tend to reduce the useful life of the photoreceptor, or limit the range of environments and printing apparatus in which the photoreceptor can be used.

## SUMMARY

This disclosure addresses some or all of the above problems, and others, by providing novel, improved photoreceptor overcoat layers. The overcoat layers generally include, as a binder material, a polyester-polyol or acrylated polyol, and a hole transporting molecule. The polyester-polyol or acrylated polyol, can be mixed with suitable crosslinking materials such as crosslinking agents and/or catalysts, to form the overcoating layer.

More particularly, in embodiments, the present disclosure provides an electrophotographic imaging member comprising:

55 a substrate,  
a charge generating layer,  
a charge transport layer, and  
an overcoating layer, said overcoating layer comprising a cured polyester polyol or cured acrylated polyol film forming resin and a charge transport material.

The present disclosure also provides electrographic image development devices comprising such electrophotographic imaging members. Also provided are imaging processes using such electrophotographic imaging members.

65 Further, the present disclosure also provides a process for forming an electrophotographic imaging member comprising:

providing an electrophotographic imaging member comprising a substrate, a charge generating layer, and a charge transport layer, and

forming thereover an overcoating layer comprising a cured polyester polyol or cured acrylated polyol film forming resin and a charge transport material.

In embodiments, the forming step can comprise providing a solution comprising said polyester polyol or acrylated polyol and said charge transport material, in a solvent; coating said solution on said electrophotographic imaging member; and crosslinking said polyester polyol or acrylated polyol to form a cured polymeric film.

#### DETAILED DESCRIPTION OF PREFERRED EMBODIMENTS

Electrophotographic imaging members are well known in the art. Electrophotographic imaging members may be prepared by any suitable technique. Typically, a flexible or rigid substrate is provided with an electrically conductive surface. A charge generating layer is then applied to the electrically conductive surface. A charge blocking layer may optionally be applied to the electrically conductive surface prior to the application of a charge generating layer. If desired, an adhesive layer may be utilized between the charge blocking layer and the charge generating layer. Usually the charge generation layer is applied onto the blocking layer and a charge transport layer is formed on the charge generation layer. This structure may have the charge generation layer on top of or below the charge transport layer.

The substrate may be opaque or substantially transparent and may comprise any suitable material having the required mechanical properties. Accordingly, the substrate may comprise a layer of an electrically non-conductive or conductive material such as an inorganic or an organic composition. As electrically non-conducting materials there may be employed various resins known for this purpose including polyesters, polycarbonates, polyamides, polyurethanes, and the like which are flexible as thin webs. An electrically conducting substrate may be any metal, for example, aluminum, nickel, steel, copper, and the like or a polymeric material, as described above, filled with an electrically conducting substance, such as carbon, metallic powder, and the like or an organic electrically conducting material. The electrically insulating or conductive substrate may be in the form of an endless flexible belt, a web, a rigid cylinder, a sheet and the like. The thickness of the substrate layer depends on numerous factors, including strength desired and economical considerations. Thus, for a drum, this layer may be of substantial thickness of, for example, up to many centimeters or of a minimum thickness of less than a millimeter. Similarly, a flexible belt may be of substantial thickness, for example, about 250 micrometers, or of minimum thickness less than 50 micrometers, provided there are no adverse effects on the final electrophotographic device.

In embodiments where the substrate layer is not conductive, the surface thereof may be rendered electrically conductive by an electrically conductive coating. The conductive coating may vary in thickness over substantially wide ranges depending upon the optical transparency, degree of flexibility desired, and economic factors. Accordingly, for a flexible photoresponsive imaging device, the thickness of the conductive coating may be between about 20 angstroms to about 750 angstroms, and more preferably from about 100 angstroms to about 200 angstroms for an optimum combination of electrical conductivity, flexibility and light transmission. The flexible conductive coating may be an electri-

cally conductive metal layer formed, for example, on the substrate by any suitable coating technique, such as a vacuum depositing technique or electrodeposition. Typical metals include aluminum, zirconium, niobium, tantalum, vanadium and hafnium, titanium, nickel, stainless steel, chromium, tungsten, molybdenum, and the like.

An optional hole blocking layer may be applied to the substrate. Any suitable and conventional blocking layer capable of forming an electronic barrier to holes between the 10 adjacent photoconductive layer and the underlying conductive surface of a substrate may be utilized.

An optional adhesive layer may be applied to the hole blocking layer. Any suitable adhesive layer well known in the art may be utilized. Typical adhesive layer materials 15 include, for example, polyesters, polyurethanes, and the like. Satisfactory results may be achieved with adhesive layer thickness between about 0.05 micrometer (500 angstroms) and about 0.3 micrometer (3,000 angstroms). Conventional techniques for applying an adhesive layer coating mixture to 20 the charge blocking layer include spraying, dip coating, roll coating, wire wound rod coating, gravure coating, Bird applicator coating, and the like. Drying of the deposited coating may be effected by any suitable conventional technique such as oven drying, infra red radiation drying, air 25 drying and the like.

At least one electrophotographic imaging layer is formed on the adhesive layer, blocking layer or substrate. The electrophotographic imaging layer may be a single layer that performs both charge generating and charge transport functions as is well known in the art or it may comprise multiple 30 layers such as a charge generator layer and charge transport layer. Charge generator layers may comprise amorphous films of selenium and alloys of selenium and arsenic, tellurium, germanium and the like, hydrogenated amorphous 35 silicon and compounds of silicon and germanium, carbon, oxygen, nitrogen and the like fabricated by vacuum evaporation or deposition. The charge generator layers may also comprise inorganic pigments of crystalline selenium and its alloys; Group II-VI compounds; and organic pigments such 40 as quinacridones, polycyclic pigments such as dibromo anthranthrone pigments, perylene and perinone diamines, polynuclear aromatic quinones, azo pigments including bis-, tris- and tetrakisazos; and the like dispersed in a film forming polymeric binder and fabricated by solvent coating 45 techniques.

Phthalocyanines have been employed as photogenerating materials for use in laser printers utilizing infrared exposure systems. Infrared sensitivity is required for photoreceptors exposed to low cost semiconductor laser diode light exposure devices. The absorption spectrum and photosensitivity of the phthalocyanines depend on the central metal atom of the compound. Many metal phthalocyanines have been 50 reported and include, oxyvanadium phthalocyanine, chloro-aluminum phthalocyanine, copper phthalocyanine, oxytitani- 55 um phthalocyanine, chlorogallium phthalocyanine, hydroxygallium phthalocyanine magnesium phthalocyanine and metal-free phthalocyanine. The phthalocyanines exist in many crystal forms which have a strong influence on photogeneration.

Any suitable polymeric film forming binder material may be employed as the matrix in the charge generating (photogenerating) binder layer. Typical polymeric film forming materials include those described, for example, in U.S. Pat. No. 3,121,006, the entire disclosure of which is incorporated herein by reference. Thus, typical organic polymeric film forming binders include thermoplastic and thermosetting resins such as polycarbonates, polyesters, polyamides, poly-

urethanes, polystyrenes, polyarylethers, polyarylsulfones, polybutadienes, polysulfones, polyethersulfones, polyethylenes, polypropylenes, polyimides, polymethylpentenes, polyphenylene sulfides, polyvinyl acetate, polysiloxanes, polyacrylates, polyvinyl acetals, polyamides, polyimides, amino resins, phenylene oxide resins, terephthalic acid resins, phenoxy resins, epoxy resins, phenolic resins, polystyrene and acrylonitrile copolymers, polyvinylchloride, vinylchloride and vinyl acetate copolymers, acrylate copolymers, alkyd resins, cellulosic film formers, poly(amideimide), styrenebutadiene copolymers, vinylidenechloride-vinylchloride copolymers, vinylacetate-vinylidenechloride copolymers, styrene-alkyd resins, polyvinylcarbazole, and the like. These polymers may be block, random or alternating copolymers.

The photogenerating composition or pigment is present in the resinous binder composition in various amounts. Generally, however, from about 5 percent by volume to about 90 percent by volume of the photogenerating pigment is dispersed in about 10 percent by volume to about 95 percent by volume of the resinous binder, and preferably from about 20 percent by volume to about 30 percent by volume of the photogenerating pigment is dispersed in about 70 percent by volume to about 80 percent by volume of the resinous binder composition. In one embodiment about 8 percent by volume of the photogenerating pigment is dispersed in about 92 percent by volume of the resinous binder composition. The photogenerator layers can also be fabricated by vacuum sublimation in which case there is no binder.

Any suitable and conventional technique may be utilized to mix and thereafter apply the photogenerating layer coating mixture. Typical application techniques include spraying, dip coating, roll coating, wire wound rod coating, vacuum sublimation and the like. For some applications, the generator layer may be fabricated in a dot or line pattern. Removing of the solvent of a solvent coated layer may be effected by any suitable conventional technique such as oven drying, infrared radiation drying, air drying and the like.

The charge transport layer may comprise a charge transporting small molecule dissolved or molecularly dispersed in a film forming electrically inert polymer such as a polycarbonate. The term "dissolved" as employed herein is defined herein as forming a solution in which the small molecule is dissolved in the polymer to form a homogeneous phase. The expression "molecularly dispersed" is used herein is defined as a charge transporting small molecule dispersed in the polymer, the small molecules being dispersed in the polymer on a molecular scale. Any suitable charge transporting or electrically active small molecule may be employed in the charge transport layer. The expression charge transporting "small molecule" is defined herein as a monomer that allows the free charge photogenerated in the transport layer to be transported across the transport layer. Typical charge transporting small molecules include, for example, pyrazolines such as 1-phenyl-3-(4'-diethylamino styryl)-5-(4"-diethylamino phenyl)pyrazoline, diamines such as N,N'-diphenyl-N,N'-bis(3-methylphenyl)-(1,1'-biphenyl)-4,4'-diamine, hydrazones such as N-phenyl-N-methyl-3-(9-ethyl)carbazyl hydrazone and 4-diethylamino benzaldehyde-1,2-diphenyl hydrazone, and oxadiazoles such as 2,5-bis (4-N,N'-diethylaminophenyl)-1,2,4-oxadiazole, stilbenes and the like. As indicated above, suitable electrically active small molecule charge transporting compounds are dissolved or molecularly dispersed in electrically inactive polymeric film forming materials. A small molecule charge transporting compound that permits injection of holes from the pigment into the charge generating layer with

high efficiency and transports them across the charge transport layer with very short transit times is N,N'-diphenyl-N,N'-bis(3-methylphenyl)-(1,1'-biphenyl)-4,4'-diamine. If desired, the charge transport material in the charge transport layer may comprise a polymeric charge transport material or a combination of a small molecule charge transport material and a polymeric charge transport material.

Any suitable electrically inactive resin binder insoluble in the alcohol solvent used to apply the overcoat layer may be employed in the charge transport layer. Typical inactive resin binders include polycarbonate resin, polyester, polyarylate, polysulfone, and the like. Molecular weights can vary, for example, from about 20,000 to about 150,000. Preferred binders include polycarbonates such as poly(4,4'-isopropylidene-diphenylene)carbonate (also referred to as bisphenol-A-polycarbonate, poly(4,4'-cyclohexylidene-diphenylene) carbonate (referred to as bisphenol-Z polycarbonate), poly(4,4'-isopropylidene-3,3'-dimethyl-diphenyl) carbonate (also referred to as bisphenol-C-polycarbonate) and the like. Any suitable charge transporting polymer may also be utilized in the charge transporting layer. The charge transporting polymer should be insoluble in any solvent employed to apply the subsequent overcoat layer described below, such as an alcohol solvent. These electrically active charge transporting polymeric materials should be capable of supporting the injection of photogenerated holes from the charge generation material and be incapable of allowing the transport of these holes therethrough.

Any suitable and conventional technique may be utilized to mix and thereafter apply the charge transport layer coating mixture to the charge generating layer. Typical application techniques include spraying, dip coating, roll coating, wire wound rod coating, and the like. Drying of the deposited coating may be effected by any suitable conventional technique such as oven drying, infra red radiation drying, air drying and the like.

Generally, the thickness of the charge transport layer is between about 10 and about 50 micrometers, but thicknesses outside this range can also be used. The hole transport layer should be an insulator to the extent that the electrostatic charge placed on the hole transport layer is not conducted in the absence of illumination at a rate sufficient to prevent formation and retention of an electrostatic latent image thereon. In general, the ratio of the thickness of the hole transport layer to the charge generator layers is preferably maintained from about 2:1 to 200:1 and in some instances as great as 400:1. The charge transport layer, is substantially non-absorbing to visible light or radiation in the region of intended use but is electrically "active" in that it allows the injection of photogenerated holes from the photoconductive layer, i.e., charge generation layer, and allows these holes to be transported through itself to selectively discharge a surface charge on the surface of the active layer.

To improve photoreceptor wear resistance, a protective overcoat layer is provided over the charge transport layer. The overcoat layer generally includes at least a film-forming resin and a hole transporting molecule. The overcoating layer can be formed, for example, from a solution or other suitable mixture of the film-forming resin and hole transporting molecule, and other optional additives.

The film-forming resin used in forming the overcoating layer is specifically a polyester polyol or acrylated polyol, preferably a highly branched polyester polyol or acrylated polyol. By "highly branched" is meant a prepolymer synthesized using a significant amount of trifunctional alcohols, such as triols, to form a polymer having a significant number of branches off of the main polymer chain. This is distin-

guished from a linear prepolymer that contains only difunctional monomers, and thus little or no branches off of the main polymer chain. As used herein, "polyester polyol" is meant to encompass such compounds that include multiple ester groups as well as multiple alcohol (hydroxyl) groups in the molecule, and which can include other groups such as, for example, ether groups and the like. In embodiments, the polyester polyol can thus include ether groups, or can be free of ether groups. Likewise, as used herein, "acrylated polyol" is meant to encompass such compounds that include multiple ether groups as well as multiple alcohol (hydroxyl) groups in the molecule, and which can include acrylate groups such as, for example, methacrylate groups and the like.

It has been found that such polyester polyols and acrylated polyols provide improved results when incorporated as a binder in the overcoating layer. Specifically, the polyester polyols and acrylated polyols provide hard binder layers, but which layers remain flexible and are not prone to crack formation.

Examples of such suitable polyester polyols include, for example, polyester polyols formed from the reaction of a polycarboxylic acid such as a dicarboxylic acid or a tricarboxylic acid (including acid anhydrides) with a polyol such as a diol or a triol. Preferably, the number of ester and alcohol groups, and the relative amount and type of polyacid and polyol, should be selected such that the resulting polyester polyol compound retains a number of free hydroxyl groups, which can be used for subsequent crosslinking of the material in forming the overcoating layer binder material. For example, suitable polycarboxylic acids include, but are not limited to, adipic acid ( $\text{COOH}[\text{CH}_2]_4\text{COOH}$ ), pimelic acid ( $\text{COOH}[\text{CH}_2]_5\text{COOH}$ ), suberic acid ( $\text{COOH}[\text{CH}_2]_6\text{COOH}$ ), azelaic acid ( $\text{COOH}[\text{CH}_2]_7\text{COOH}$ ), sebasic acid ( $\text{COOH}[\text{CH}_2]_8\text{COOH}$ ), and the like. Suitable polyols include, but are not limited to, difunctional materials such as glycols or trifunctional alcohols such as triols and the like, including propanediols ( $\text{HO}[\text{CH}_2]_3\text{OH}$ ), butanediols ( $\text{HO}[\text{CH}_2]_4\text{OH}$ ), hexanediols ( $\text{HO}[\text{CH}_2]_6\text{OH}$ ), glycerine ( $\text{HOCH}_2\text{CHOHCH}_2\text{OH}$ ), 1,2,6-Hexane triol ( $\text{HOCH}_2\text{CHOH}[\text{CH}_2]_4\text{OH}$ ), and the like.

In embodiments, the suitable polyester polyols are reaction products of polycarboxylic acids and polyols and can be represented by the following formula (1):



where  $\text{R}_a$  and  $\text{R}_c$  independently represent linear alkyl groups or branched alkyl groups derived from the polyols, the alkyl groups having from 1 to about 20 carbon atoms;  $\text{R}_b$  and  $\text{R}_d$  independently represent alkyl groups derived from the polycarboxylic acids, the alkyl groups having from 1 to about 20 carbon atoms; and  $m$ ,  $n$ ,  $p$ , and  $q$  represent mole fractions of from 0 to 1, such that  $n+m+p+q=1$ .

Specific commercially available examples of such suitable polyester polyols include, for example: the DESMOPHEN® series of products available from Bayer Chemical, including the DESMOPHEN® 800, 1110, 1112, 1145, 1150, 1240, 1262, 1381, 1400, 1470, 1630, 2060, 2061, 2062, 3060, 4027, 4028, 404, 4059, 5027, 5028, 5029, 5031, 5035, and 5036 products; the SOVERMOL® series of products available from Cognis, including the SOVERMOL® 750, 805, 815, 908, 910, and 913 products; and the HYDAGEN® series of products available from Cognis, including the HYDAGEN® HSP product; and mixtures thereof. Particularly preferred in embodiments are DES-

MOPHEN® 800 and SOVERMOL® 750, or mixtures thereof. DESMOPHEN® 800 is a highly branched polyester bearing hydroxyl groups, having an acid value of  $\leq 4$  mg KOH/g, a hydroxyl content of about  $8.6\pm 0.3\%$ , and an equivalent weight of about 200. DESMOPHEN® 800 corresponds to the above formula (1) where the polymer contains 50 parts adipic acid, 10 parts phthalic anhydride, and 40 parts 1,2,6-hexanetriol, where  $\text{R}_b=[\text{CH}_2]_4-$ ,  $n=0.5$ ,  $\text{R}_d=1,2-\text{C}_6\text{H}_4-$ ,  $q=0.1$ ,  $\text{R}_a=\text{R}_c=\text{CH}_2-\text{[CHO}-$   $[\text{CH}_2]_4-$ , and  $m+p=0.4$ . DESMOPHEN® 1100 corresponds to the above formula (1) where the polymer contains 60 parts adipic acid, 40 parts 1,2,6-hexanetriol, and 60 parts 1,4-butanediol, where  $\text{R}_b=\text{R}_d=[\text{CH}_2]_4-$ ,  $n+q=0.375$ ,  $\text{R}_a=\text{CH}_2-\text{[CHO}-$   $[\text{CH}_2]_4-$ ,  $m=0.25$ ,  $\text{R}_c=[\text{CH}_2]_4-$ , and  $p=0.375$ . SOVERMOL® 750 is a branched polyether/polyester/polyol having an acid value of  $\leq 2$  mg KOH/g, and a hydroxyl value of 300-330 mg KOH/g.

In other embodiments, the film-forming resin can be an acrylated polyol. Suitable acrylated polyols can be, for example, the reaction products of propylene oxide modified with ethylene oxide, glycols, triglycerol and the like. These polyols are further reacted with substituted acrylic acids, alcohol containing acrylates, substituted acryloyl chlorides, and the like, forming terminal acrylate groups. Such acrylated polyols can be represented by the following formula (2):



where  $\text{R}_t$  represent  $\text{CH}_2\text{CR}_1\text{CO}_2-$  where  $\text{R}_1$  is an alkyl group of from 1 to about 20 carbon atoms or more such as methyl, ethyl, and the like and where  $t$  represents mole fractions of acrylated sites from 0 to 1.  $\text{R}_a$  and  $\text{R}_c$ , independently represent linear alkyl/alkoxy groups or branched alkyl/alkoxy groups derived from the polyols, the alkyl/alkoxy groups having from 1 to about 20 carbon atoms;  $\text{R}_b$  and  $\text{R}_d$  independently represent alkyl/alkoxy groups, the alkyl/alkoxy groups having from 1 to about 20 carbon atoms; and  $m$ ,  $n$ ,  $p$ , and  $q$  represent mole fractions of from 0 to 1, such that  $n+m+p+q=1$ . In formula (2), the notation "[ $\text{R}_t-\text{CH}_2-$ ] $_t$ " indicates that the acrylate groups react with some of the hydroxyl groups in the main chain or branches of the polyol component.

In forming the binder material for the overcoating layer, any suitable crosslinking agents, catalysts, and the like can be included in known amounts for known purposes. For example, it is particularly preferred in embodiments that a crosslinking agent or accelerator, such as a melamine crosslinking agent or accelerator, be included with the polyester polyol or acrylated polyol for forming the overcoating layer. Incorporation of a crosslinking agent or accelerator provides reaction sites to interact with the polyester polyol or acrylated polyol, to provide a branched, crosslinked structure. When so incorporated, any suitable crosslinking agent or accelerator can be used, including, for example, trioxane, melamine compounds, and mixtures thereof. Where melamine compounds are used, they can be suitable functionalized to be, for example, melamine formaldehyde, methoxymethylated melamine compounds, such as glycourlformaldehyde and benzoguanamine-formaldehyde, and the like. An example of a suitable methoxymethylated melamine compound is Cymel 303 (available from Cytec Industries), which is a methoxymethylated melamine

11

compound with the formula  $(\text{CH}_3\text{OCH}_2)_6\text{N}_3\text{C}_3\text{N}_3$  and the following structure:



Crosslinking is generally accomplished by heating in the presence of a catalyst. Thus, the solution of the polyester polyol or acrylated polyol can also preferably include a suitable catalyst. Any suitable catalyst may be employed. Typical catalysts include, for example, oxalic acid, maleic acid, carbollylic acid, ascorbic acid, malonic acid, succinic acid, tartaric acid, citric acid, p-toluenesulfonic acid, methanesulfonic acid, and the like and mixtures thereof.

If desired or necessary, a blocking agent can also be included. A blocking agent can be used to "tie up" or block the acid effect to provide solution stability until the acid catalyst function is desired. Thus, for example, the blocking agent can block the acid effect until the solution temperature is raised above a threshold temperature. For example, some blocking agents can be used to block the acid effect until the solution temperature is raised above about 100° C. At that time, the blocking agent dissociates from the acid and vaporizes. The unassociated acid is then free to catalyze the polymerization. Examples of such suitable blocking agents include, but are not limited to, pyridine and commercial acid solutions containing blocking agents such as Cycat 4040 available from Cytec Ind.

The temperature used for crosslinking varies with the specific catalyst and heating time utilized and the degree of crosslinking desired. Generally, the degree of crosslinking selected depends upon the desired flexibility of the final photoreceptor. For example, complete crosslinking may be used for rigid drum or plate photoreceptors. However, partial crosslinking is preferred for flexible photoreceptors having, for example, web or belt configurations. The degree of crosslinking can be controlled by the relative amount of catalyst employed. The amount of catalyst to achieve a desired degree of crosslinking will vary depending upon the specific coating solution materials, such as polyol, catalyst, temperature and time used for the reaction. Preferably, the polyol is cross linked at a temperature between about 100° C. and about 150° C. A typical cross linking temperature used for polyols with *p*-toluenesulfonic acid as a catalyst is less than about 140° C. for about 40 minutes. A typical concentration of acid catalyst is between about 0.01 and about 5.0 weight percent based on the weight of polyol. After crosslinking, the overcoating should be substantially insoluble in the solvent in which it was soluble prior to crosslinking. Thus, no overcoating material will be removed when rubbed with a cloth soaked in the solvent. Crosslinking results in the development of a three dimensional network which restrains the transport molecule in the crosslinked polymer network.

Any suitable alcohol solvent may be employed for the film forming polymers. Typical alcohol solvents include, for example, butanol, propanol, methanol, 1-methoxy-2-propanol, and the like and mixtures thereof. Other suitable solvents that can be used in forming the overcoating layer

12

solution include, for example, tetrahydrofuran, monochlorobenzene, and mixtures thereof. These solvents can be used in addition to, or in place of, the above alcohol solvents, or they can be omitted entirely. However, in some embodiments, it is preferred that higher boiling alcohol solvents be avoided, as they can interfere with the desired cross-linking reaction.

Any suitable hole transport material may be utilized in the overcoating layer. Preferably, the hole transport material is an alcohol soluble polyhydroxy diaryl amine small molecule charge transport material having at least two hydroxy functional groups. An especially preferred small molecule hole transporting material can be represented by the following formula:



wherein:

25 m is 0 or 1,

Z is selected from the group consisting of:



n is 1 or 1.

Ar is selected from the group consisting of:



R is selected from the group consisting of  $-\text{CH}_3$ ,  $-\text{C}_2\text{H}_5$ ,  $-\text{C}_3\text{H}_7$ , and  $-\text{C}_4\text{H}_9$ ,

Ar' is selected from the group consisting of:





X is selected from the group consisting of:



s is 0,1 or 2,

the dihydroxy arylamine compound preferably being free of any direct conjugation between the —OH groups and the nearest nitrogen atom through one or more aromatic rings.

The expression "direct conjugation" is defined as the presence of a segment, having the formula  $-(C=C)_n-C=C-$  in one or more aromatic rings directly between an  $-OH$  group and the nearest nitrogen atom. Examples of direct conjugation between the  $-OH$  groups and the nearest nitrogen atom through one or more aromatic rings include a compound containing a phenylene group having an  $-OH$  group in the ortho or para position (or 2 or 4 position) on the phenylene group relative to a nitrogen atom attached to the phenylene group or a compound containing a polyphenylene group having an  $-OH$  group in the ortho or para position on the terminal phenylene group relative to a nitrogen atom attached to an associated phenylene group.

Typical polyhydroxy arylamine compounds utilized in the overcoat of embodiments include, for example: N,N'-diphenyl-N,N'-bis(3-hydroxyphenyl)-[1,1'-biphenyl]-4,4'-diamine; N,N,N',N'-tetra(3-hydroxyphenyl)-[1,1'-biphenyl]-4,4'-diamine; N,N-di(3-hydroxyphenyl)-m-toluidine; 1,1-bis-[4-(di-N,N-m-hydroxyphenyl)-aminophenyl]-cyclohexane; 1,1-bis[4-(N-m-hydroxyphenyl)-4-(N-phenyl)-aminophenyl]-cyclohexane; bis-(N-(3-hydroxyphenyl)-N-phenyl-4-aminophenyl)-methane; bis[(N-(3-hydroxyphenyl)-N-phenyl)-4-aminophenyl]-isopropylidene; N,N'-diphenyl-N,N'-bis(3-hydroxyphenyl)-[1,1'4',1"-terphenyl]-4,4"-diamine; 9-ethyl-3,6-bis[N-phenyl-N-3-(3-hydroxyphenyl)-amino]-carbazole; 2,7-bis[N,N-di(3-hydroxyphenyl)-amino]-fluorene; 1,6-bis[N,N-di(3-hydroxyphenyl)-amino]-pyrene; 1,4-bis[N-phenyl-N-(3-hydroxyphenyl)]-phenylenediamine.

The thickness of the continuous overcoat layer selected depends upon the abrasiveness of the charging (e.g., bias charging roll), cleaning (e.g., blade or web), development (e.g., brush), transfer (e.g., bias transfer roll), etc., in the system employed and can range from about 1 or about 2 microns up to about 10 or about 15 microns or more. A thickness of between about 1 micrometer and about 5 micrometers in thickness is preferred, in embodiments. Typical application techniques include spraying, dip coat-

ing, roll coating, wire wound rod coating, and the like. Drying of the deposited coating may be effected by any suitable conventional technique such as oven drying, infrared radiation drying, air drying and the like. The dried 5 overcoating of this disclosure should transport holes during imaging and should not have too high a free carrier concentration. Free carrier concentration in the overcoat increases the dark decay. Preferably the dark decay of the overcoated layer should be about the same as that of the 10 unovercoated device.

In the dried overcoating layer, the composition can include from about 10 to about 90 percent by weight film-forming binder, and from about 90 to about 10 percent by weight hole transporting molecule. For example, in 15 embodiments, the hole transporting molecule can be incorporated into the overcoating layer in an amount of from about 20 to about 70 percent by weight, such as about 33 percent by weight. As desired, the overcoating layer can also include other materials, such as conductive fillers, abrasion 20 resistant fillers, and the like, in any suitable and known amounts.

Advantages provided by the present disclosure include, in embodiments, overcoating layers that are hard yet flexible. Some traditional overcoat layers are hard but inflexible, resulting in crack formation during flexing and use. This problem is exacerbated by exposure of the overcoating layers to corona discharge, a necessary part of electrostatographic printing. Corona discharge can increase the crack rate of the overcoating layers, resulting in shortened lifetime and poor image formation. However, in embodiments, the present disclosure provides hard yet flexible overcoating layers. These overcoating layers are hard, which means that they can withstand wear to a great extent, but they are also flexible, meaning that they can resist cracking during flexing and under corona exposure. A further benefit of the overcoating layers is that they can be electrically transparent, meaning that additional changes to the photoreceptor are not required in order to incorporate the disclosed overcoating layers.

40 A further advantage, in embodiments, is that the over-coating layer, and thus the entire imaging member structure, are less sensitive to atmospheric moisture. Lower moisture sensitivity allows the imaging member to perform more predictably, and more uniformly, in different temperature/humidity environments.

Also, included within the scope of the present disclosure are methods of imaging and printing with the imaging members illustrated herein. These methods generally involve the formation of an electrostatic latent image on the imaging member; followed by developing the image with a toner composition comprised, for example, of thermoplastic resin, colorant, such as pigment, charge additive, and surface additives, reference U.S. Pat. Nos. 4,560,635, 4,298,697 and 4,338,390, the disclosures of which are totally incorporated herein by reference; subsequently transferring the image to a suitable substrate; and permanently affixing the image thereto. In those environments wherein the device is to be used in a printing mode, the imaging method involves the same steps with the exception that the exposure step can be accomplished with a laser device or image bar.

An example is set forth hereinbelow and is illustrative of different compositions and conditions that can be utilized in practicing the disclosure. All proportions are by weight unless otherwise indicated. It will be apparent, however, that the disclosure can be practiced with many types of compositions and can have many different uses in accordance with the disclosure above and as pointed out hereinafter.

## 15

## EXAMPLES

## Example 1

## Preparation of Overcoating Composition

A coating composition is formed containing 4 grams DESMOPHEN® 800 polyester polyol, 2.4 grams Cymel 1130, 18 grams 1-methoxy-2-propanol (Dowanol), and 3.2 grams N,N'-diphenyl-N,N'-bis(3-hydroxyphenyl)-[1,1'-biphenyl]-4,4'-diamine in a 1 ounce bottle. The components are mixed and the temperature is raised to about 40° C. until a complete solution is achieved. Next, 0.9 grams of p-toluenesulfonic acid/pyridine (8% acid/2% pyridine in 1-methoxy-2-propanol) (0.072 grams acid, 0.75% by weight) as catalyst is added

## Example 2

## Preparation of Overcoated Imaging Member

An overcoated imaging member sheet or belt is formed using the coating composition of Example 1. In particular, an electrophotographic imaging member web stock is prepared by providing a 0.02 micrometer thick titanium layer coated on a biaxially oriented polyethylene naphthalate substrate (Kadalex, available from ICI Americas, Inc.) having a thickness of 3.5 mils (89 micrometers) and applying thereto, using a gravure coating technique and a solution containing 10 grams gamma aminopropyltriethoxy silane, 10.1 grams distilled water, 3 grams acetic acid, 684.8 grams of 200 proof denatured alcohol and 200 grams heptane. This layer is then allowed to dry for 5 minutes at 135° C. in a forced air oven. The resulting blocking layer has an average dry thickness of 0.05 micrometer measured with an ellipsometer.

An adhesive interface layer is then prepared by applying with extrusion process to the blocking layer a wet coating containing 5 percent by weight based on the total weight of the solution of polyester adhesive (Mor-Ester 49,000, available from Morton International, Inc.) in a 70:30 volume ratio mixture of tetrahydrofuran:cyclohexanone. The adhesive interface layer is allowed to dry for 5 minutes at 135° C. in a forced air oven. The resulting adhesive interface layer has a dry thickness of 0.065 micrometer

The adhesive interface layer is thereafter coated with a photogenerating layer. The photogenerating layer dispersion is prepared by introducing 0.45 grams of lupilon 200 (PC-Z 200) available from Mitsubishi Gas Chemical Corp and 50 ml of tetrahydrofuran into a 4 oz. glass bottle. To this solution is added 2.4 grams of hydroxygallium phthalocyanine and 300 grams of 1/8 inch (3.2 millimeter) diameter stainless steel shot. This mixture is then placed on a ball mill for 20 to 24 hours. Subsequently, 2.25 grams of PC-Z 200 is dissolved in 46.1 gm of tetrahydrofuran, then added to this OHGaPc slurry. This slurry is then placed on a shaker for 10 minutes. The resulting slurry is, thereafter, coated onto the adhesive interface by an extrusion application process to form a layer having a wet thickness of 0.25 mil. However, a strip about 10 mm wide along one edge of the substrate web bearing the blocking layer and the adhesive layer is deliberately left uncoated by any of the photogenerating layer material to facilitate adequate electrical contact by the ground strip layer that is applied later. This photogenerating layer is dried at 135° C. for 5 minutes in a forced air oven to form a dry thickness photogenerating layer having a thickness of 0.4 micrometer layer.

## 16

This coated imaging member web is simultaneously overcoated with a charge transport layer and a ground strip layer using extrusion co-coating process. The charge transport layer is prepared by introducing into an amber glass bottle a weight ratio of 1:1 N,N'-diphenyl-N,N'-bis(3-methylphenyl)-1,1'-biphenyl-4-4'-diamine, and Makrolon 5705, a polycarbonate resin having a weight average molecular weight of about 120,000 commercially available from Bayer A. G. The resulting mixture is dissolved to give a 15 percent by weight solid in 85 percent by weight methylene chloride. This solution is applied onto the photogenerator layer to form a coating which upon drying has a thickness of 29 micrometers.

The approximately 10 mm wide strip of the adhesive layer left uncoated by the photogenerator layer is coated over with a ground strip layer during the co-coating process. This ground strip layer, after drying along with the co-coated charge transport layer at 135° C. in the forced air oven for minutes, has a dried thickness of about 19 micrometers. This ground strip is electrically grounded, by conventional means such as a carbon brush contact means during conventional xerographic imaging process.

An anticurl coating is prepared by combining 8.82 grams of polycarbonate resin (Makrolon 5705, available from Bayer AG), 0.72 gram of polyester resin (Vitel PE-200, available from Goodyear Tire and Rubber Company) and 90.1 grams of methylene chloride in a glass container to form a coating solution containing 8.9 percent solids. The container is covered tightly and placed on a roll mill for about 24 hours until the polycarbonate and polyester are dissolved in the methylene chloride to form the anticurl coating solution. The anticurl coating solution is then applied to the rear surface (side opposite the photogenerator layer and charge transport layer) of the imaging member web stock, again by extrusion coating process, and dried at 135° C. for about 5 minutes in the forced air oven to produce a dried film thickness of about 17 micrometers.

The sheet is overcoated with the overcoat layer composition of Example 1. The coating composition is applied using a 0.125 mil Bird bar applicator and dried at 125° C. for 4 minutes. The result is an imaging member having an overcoating layer thickness of 3 microns.

## Comparative Example 2

## Preparation of Overcoated Imaging Member

An imaging member is made in the same manner as in Example 2, except that the overcoating layer is omitted.

## Example 3

## Testing of Imaging Members

The imaging members of Example 2 and Comparative Example 2 are tested for their electrostatographic sensitivity and cycling stability in a scanner. In the scanner, each photoreceptor sheet to be evaluated is mounted on a cylindrical aluminum drum substrate that is rotated on a shaft. The devices are charged by a corotron mounted along the periphery of the drum. The surface potential is measured as a function of time by capacitively coupled voltage probes placed at different locations around the shaft. The probes are calibrated by applying known potentials to the drum substrate. Each photoreceptor sheet on the drum is exposed to a light source located at a position near the drum downstream from the corotron. As the drum is rotated, the initial

17

(pre-exposure) charging potential is measured by voltage probe 1. Further rotation leads to an exposure station, where the photoreceptor device is exposed to monochromatic radiation of a known intensity. The devices are erased by a light source located at a position upstream of charging. The measurements illustrated in the Table below include the charging of each photoconductor device in a constant current or voltage mode. The devices are charged to a negative polarity corona. The surface potential after exposure is measured by a second voltage probe. The devices are finally exposed to an erase lamp of appropriate intensity and any residual potential is measured by a third voltage probe. The process is repeated with the magnitude of the exposure automatically changed during the next cycle. The photodischarge characteristics are obtained by plotting the potentials at voltage probe 2 as a function of light exposure. The following results show that there is no significant difference between the imaging member having no overcoat (Comparative Example 2) and the imaging member having an overcoat (Example 2).

| # cycles | Example | V(1.5) | V(2.5) | V(6) | V(3.5) |
|----------|---------|--------|--------|------|--------|
| 0        | 2       | 72     | 34     | 19   | 28     |
|          | Comp. 2 | 79     | 46     | 29   | 41     |
| 10,000   | 2       | 111    | 66     | 38   | 57     |
|          | Comp. 2 | 141    | 100    | 68   | 89     |

Next, the imaging members of Example 2 and Comparative Example 2 are tested for corona sensitivity. Hand-coated samples of the formulations described in Example 2 and Comparative example 2 are cut into small sheets (1.5 inches×11 inches) and wrapped around a 84 mm photoreceptor drum. This drum with the sample belt wrapping around it is then exposed to corona effluents generated from a charging device. After being exposed for 30 minutes, using a DC 12 Limoges printer, the drum is printed with a target containing various types of bit lines for LCM deletion. The target print has 5 different bit lines ranging from 1 bit to 5 bit. The sample with the least number of visible lines is badly affected by corona effluents and completely deleted if there are no visible lines. The results show that after being exposed to corona effluent for 30 minutes, the imaging member having no overcoat (Comparative Example 2) has no visible printed bit lines, whereas the imaging member having an overcoat (Example 2) shows all of its bit lines during printing.

Next, the imaging members of Example 2 and Comparative Example 2 are tested for scratch resistance, by abrading the imaging members with toner carrier beads. Hand-coated samples of Example 2 and Comparative Example 2 are cut into small sheets as above and are flexed in a tri-roller flexing system. Each belt is under a 1.1 lb/inch tension and each roller is 0.5 inches in diameter. A polyurethane spots blade is placed in contact with each belt at a angle between 5 to 15 degrees. Carrier beads of about 100 micrometers in size are attached to the spots blade by the aid of a double tape. Belts are flexed for 7000 cycles. The surface morphology of each imaging member is then analyzed. The following results show that the imaging member having-no overcoat (Comparative Example 2) has deeper scratches and is less resistant to abrading by the carrier beads, whereas the imaging member having an overcoat (Example 2) shows more shallow scratches and higher resistance to abrasion by the carrier beads. In the Table, Rq is the root mean square

18

roughness, Rz is 10 point mean roughness, and Rmax is maximum peak to valley height, all expressed in microns.

| Example | Rq   | Rz   | Ra   | Rmax |
|---------|------|------|------|------|
| 2       | 0.12 | 2.11 | 0.07 | 3.14 |
| Comp. 2 | 0.37 | 4.70 | 0.22 | 8.65 |

10 Lastly, the imaging members of Example 2 and Comparative Example 2 are tested for mechanical crack resistance, by flexing the belts on a tri-roller fixture with ¼ diameter rolls for 5,000 cycles before being exposed to corona effluent. The flexed and exposed areas are then printed for crack assessment. The results show that the imaging member having no overcoat (Comparative Example 2) has significantly more cracks than the imaging member having an overcoat (Example 2), and that the imaging member of Example 2 appears to be more resistant to mechanical flexing and corona effluent.

#### Example 4

##### Preparation of Polyester Polyol Overcoat

25 A coating composition is formed containing 7.0 grams SOVERMOL® 750 polyester polyol, 54 grams 1-methoxy-2-propanol (Dowanol PM), 5.0 grams Cymel 303 melamine formaldehyde crosslinking agent and 6.0 grams N,N'-diphenyl-N,N'-bis(3-hydroxyphenyl)-[1,1'-biphenyl]-4,4'-diamine in a 1 ounce bottle. The components are mixed and the temperature is raised to about 40° C. until a complete solution is achieved. Next, 1.68 grams of p-toluenesulfonic acid/pyridine (8% acid/2% pyridine in 1-methoxy-2-propanol) (0.135 grams acid, 0.75% by weight) as a catalyst is added.

#### Example 5

##### Preparation of Acrylated Polyol Overcoat

30 A coating composition is formed containing 2.5 grams Joncryl 587 [acrylated polyol from Johnson Polymers Inc.], 3.5 grams Cymel 303, 27 grams 1-methoxy-2-propanol (Dowanol PM), and 3.0 grams N,N'-diphenyl-N,N'-bis(3-hydroxyphenyl)-[1,1'-biphenyl]-4,4'-diamine in a 1 ounce bottle. The components are mixed and the temperature is raised to about 40° C. until a complete solution is achieved. Next, 0.9 grams of p-toluenesulfonic acid/pyridine (8% acid/2% pyridine in 1-methoxy-2-propanol) (0.072 grams acid, 0.75% by weight) as catalyst is added.

#### Example 6

##### Preparation of Overcoated Imaging Member

35 Electrophotographic imaging member are prepared by applying by dip coating a charge blocking-layer onto the rough surface of an aluminum drum having a diameter of 3 cm and a length of 31 cm. The blocking layer coating mixture is a solution of 8 weight percent polyamide (nylon 6) dissolved in a 92 weight percent butanol, methanol and water solvent mixture. The butanol, methanol and water mixture percentages are 55, 36 and 9 percent by weight, respectively. The coating is applied at a coating bath with 60 withdrawal rate of 300 millimeters/minute. After drying in a forced air oven, the blocking layer has a thickness of 1.5 micrometers. The dried blocking layer is coated with a

19

charge generating layer containing 2.5 weight percent hydroxy gallium phthalocyanine pigment particles, 2.5 weight percent polyvinylbutyral film forming polymer and 95 weight percent cyclohexanone solvent. The coating is applied at a coating bath withdrawal rate of 300 millimeters/minute. After drying in a forced air oven, the charge generating layer has a thickness of 0.2 micrometer. The drum is subsequently coated with a charge transport layer containing N,N'-diphenyl-N,N'-bis(3-methylphenyl)-1,1'-biphenyl-4,4'-diamine dispersed in polycarbonate binder (PCZ 300, available from the Mitsubishi Chemical Company). The charge transport coating mixture consists of 8 weight percent N,N'-diphenyl-N,N'-bis(3-methylphenyl)-1,1'-biphenyl-4,4'-diamine, 12 weight percent binder and 80 weight percent monochlorobenzene solvent. The coating is applied in a Tsukiage dip coating apparatus. After drying in a forced air oven for 45 minutes at 118° C., the transport layer has a thickness of 20 micrometers.

#### Example 7

##### Preparation of Overcoated Drum Imaging Member

A drum from Example 6 is overcoated with the overcoat solution composition from Example 4. The coating composition is applied using a Tsukiage dip coating apparatus and dried at 125° C. for 40 minutes. The result is an imaging member having an overcoating layer thickness of from about 2.5 to about 3.0 microns.

#### Example 8

##### Preparation of Overcoated Drum Imaging Member

A drum from Example 6 is overcoated with the overcoat solution composition from Example 5. The coating composition is applied using a Tsukiage dip coating apparatus and dried at 125° C. for 40 minutes. The result is an imaging member having an overcoating layer thickness of from about 2.5 to about 3.0 microns.

#### Comparative Example 9

##### Preparation of Non-Overcoated Imaging Member

An imaging member is made in the same manner as in Example 6, except that the overcoating layer is omitted.

#### Example 10

##### Testing of Imaging Members

The drums of Example 7 and 8 and Comparative Example 9 are mounted in an electrostatographic imaging scanner, a device well known in the industry and equipped with means to rotate the drum while it is electrically charged and discharged. The charge on the sample is monitored through use of electrostatic probes placed at precise positions around the circumference of the device. The samples in this Example are charged to a negative potential of 500 Volts. As the device rotates, the initial charging potential is measured by voltage probe 1. The sample is then exposed to monochromatic radiation of known intensity, and the surface potential measured by voltage probes 2 and 3. Finally, the sample is exposed to an erase lamp of appropriate intensity and wavelength and any residual potential is measured by voltage probe 4. The process is repeated under the control of the scanner's computer, and the data is stored in the computer. The PIDC (photo induced discharge curve) is obtained

20

by plotting the potentials at voltage probes 2 and 3 as a function of the light energy. The samples' dark decay and charge acceptance are also determined from the scanner data.

5 The PIDCs are measured under three different environmental conditions, e.g. A-zone (80° F., 85% humidity), B-zone (72° F., 50% humidity), and C-zone (15° F., 52% humidity). The results show that there is no significant difference between the overcoated drums of Example 7 and 8 and the non-overcoated drums of Comparative Example 9.

10 The overcoated drums of Example 7 and 8 and the non-overcoated drum of Comparative Example 9 are also subjected to a long electrical cycling test in A-zone. The results show no CDS (charge deletion spots) or background issues found during the cycling test at 2 million cycles for the overcoated drum. Instead, the occurrence of CDS occurs sometime between about 2 and 2.3 million cycles. In contrast, for the non-overcoated drum, CDS and background problems occur after only 340 to 510 cycles.

15 Next, the imaging members of Example 7 and 8 and Comparative Example 9 were tested for abrasion resistance (wear rate) in a wear fixture that includes a bias charging roll for charging. Wear rate is calculated in terms of nanometers/kilocycles of rotation (nm/kc). The wear rate for the imaging member having no overcoat (Comparative Example 9) is about 75 to 85 nm/kc, as compared to the about 10 to 15 nm/kc wear rate of the imaging member having an overcoat of either polyester or acrylic polyol (Example 7 and 8).

20 Lastly, the imaging members of Example 9 and Comparative Example 6 are tested for water repellency. The drums are placed in an A-zone chamber for 2 days. Afterwards, the imaging member is immediately printed with a XEROX® emulsion/aggregation toner composition in a loss of resolution test used to measure surface conductivity. The target image includes 1 bit and 2 bit lines and images with variations in black color intensity. The results show no indication of water absorption in the overcoat layers of Example 7 and 8, indicating no added conductivity in the overcoat layer. Image quality of the printed image is excellent.

25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650

## 21

5. The electrophotographic imaging member of claim 1, wherein the film forming resin is a polyester polyol represented by the formula:



where Ra and Rc independently represent linear alkyl groups or branched alkyl groups derived from the polyols, the alkyl groups having from 1 to about 20 carbon atoms; Rb and Rd independently represent alkyl groups derived from the polycarboxylic acids, the alkyl groups having from 1 to about 20 carbon atoms; and m, n, p, and q represent mole fractions of from 0 to 1, such that  $n+m+p+q=1$ .

6. The electrophotographic imaging member of claim 1, wherein the film forming resin is a polyester polyol that before curing is a branched polyester bearing hydroxyl groups, having an acid value of  $\leq 4$  mg KOH/g, a hydroxyl content of about  $8.6\pm 0.3\%$ , and an equivalent weight of about 200.

7. The electrophotographic imaging member of claim 1, wherein the film forming resin is a polyester polyol that before curing is a branched polyether/polyester having an acid value of  $\leq 2$  mg KOH/g, and a hydroxyl value of 300-330 mg KOH/g.

8. The electrophotographic imaging member of claim 1, wherein the film forming resin is a cured acrylated polyol.

9. The electrophotographic imaging member of claim 8, wherein the acrylated polyol is a branched acrylated polyol.

10. The electrophotographic imaging member of claim 8, wherein the acrylated polyol is represented by the formula:



where R<sub>t</sub> represent  $\text{CH}_2\text{CR}_1\text{CO}_2$ — where R<sub>1</sub> is an alkyl group of from 1 to about 20 carbon atoms; t represents mole fractions of acrylated sites from 0 to 1; Ra and Rc independently represent linear alkyl or alkoxy groups or branched alkyl or alkoxy groups derived from the polyols, the alkyl and alkoxy groups having from 1 to about 20 carbon atoms; Rb and Rd independently represent alkyl or alkoxy groups, the alkyl and alkoxy groups having from 1 to about 20 carbon atoms; and m, n, p, and q represent mole fractions of from 0 to 1, such that  $n+m+p+q=1$ .

11. The electrophotographic imaging member of claim 1, wherein the overcoating layer is formed from a solution comprising said film forming resin and said charge transport material, in a solvent.

12. The electrophotographic imaging member of claim 11, wherein the solution further comprises at least one of a crosslinking accelerator and a catalyst.

13. The electrophotographic imaging member of claim 11, wherein the solution further comprises a melamine crosslinking accelerator and an acid catalyst.

14. The electrophotographic imaging member of claim 13, wherein the crosslinking accelerator is a methoxymethylated melamine compound.

15. The electrophotographic imaging member of claim 1, wherein the overcoating layer comprising from about 0 to about 60 percent by weight charge transport material and from about 100 to about 60 percent by weight film forming resin.

16. A process for forming an electrophotographic imaging member comprising:

providing an electrophotographic imaging member comprising a substrate, a charge generating layer, and a charge transport layer, and

## 22

forming thereover an overcoating layer comprising a cured polyester polyol or cured acrylated polyol film forming resin and a charge transport material.

17. The process of claim 16, wherein the forming step comprises:

providing a solution comprising said film forming resin and said charge transport material, in a solvent; coating said solution on said electrophotographic imaging member; and crosslinking said film forming resin to form a cured polymeric film.

18. The process of claim 16, wherein the film forming resin is a branched polyester polyol.

19. The process of claim 16, wherein the film forming resin is a polyester polyol represented by the formula:



where Ra and Rc independently represent linear alkyl groups or branched alkyl groups derived from the polyols, the alkyl groups having from 1 to about 20 carbon atoms; Rb and Rd independently represent alkyl groups derived from the polycarboxylic acids, the alkyl groups having from 1 to about 20 carbon atoms; and m, n, p, and q represent mole fractions of from 0 to 1, such that  $n+m+p+q=1$ .

20. The process of claim 16, wherein the film forming resin is a polyester polyol that before curing is selected from the group consisting of:

a branched polyester bearing hydroxyl groups; having an acid value of  $\leq 4$  mg KOH/g, a hydroxyl content of about  $8.6\pm 0.3\%$ , and an equivalent weight of about 200; and

a branched polyether/polyester having an acid value of  $\leq 2$  mg KOH/g, and a hydroxyl value of 300-330 mg KOH/g.

21. The process of claim 16, wherein the film forming resin is a cured acrylated polyol represented by the formula:



where R<sub>t</sub> represent  $\text{CH}_2\text{CR}_1\text{CO}_2$ — where R<sub>1</sub> is an alkyl group of from 1 to about 20 carbon atoms; t represents mole fractions of acrylated sites from 0 to 1; Ra and Rc independently represent linear alkyl or alkoxy groups or branched alkyl or alkoxy groups derived from the polyols, the alkyl and alkoxy groups having from 1 to about 20 carbon atoms; Rb and Rd independently represent alkyl or alkoxy groups, the alkyl and alkoxy groups having from 1 to about 20 carbon atoms; and m, n, p, and q represent mole fractions of from 0 to 1, such that  $n+m+p+q=1$ .

22. The process of claim 17, wherein the solution further comprises at least one of a crosslinking accelerator and a catalyst.

23. The process of claim 17, wherein the solution further comprises a melamine crosslinking accelerator and an acid catalyst.

24. The process of claim 23, wherein the crosslinking accelerator is a methoxymethylated melamine compound.

25. An electrographic image development device, comprising an electrophotographic imaging member comprising:

a substrate,  
a charge generating layer,  
a charge transport layer, and  
an overcoating layer, said overcoating layer comprising a cured polyester polyol or cured acrylated polyol film forming resin and a charge transport material.